

1

3,280,035

## OIL COMPOSITIONS CONTAINING EMULSION-INHIBITING ACETYLENIC COMPOUNDS

Francis J. Bonner, Wilmington, Del., assignor to Mobil Oil Corporation, a corporation of New York  
No Drawing. Filed Apr. 17, 1963, Ser. No. 273,571  
4 Claims. (Cl. 252—52)

This invention relates to the inhibition of the emulsifying tendencies of additive-modified lubricating oils and to the inhibited lubricating oil compositions.

In using lubricating oils, it is found that the oils frequently become contaminated with water through leakage, condensation or the like. This is particularly true with the turbine lubricating oils which also may pick up more water from that added during in-plant reprocessing of the oil. The lubricating oils normally are compounded with various detergents, anti-rust agents, antioxidants and other additives which act as oil emulsifiers in the presence of water. It is desirable to obtain rapid separation and removal of any water dispersed in the lubricating oil and this is usually accomplished by centrifuging and/or settling. Obviously, the formation of oil-water emulsions would interfere with any such separation of the water from the oil.

It is one of the objects of the present invention to inhibit the emulsifying tendencies of lubricating oils. It is another object to enhance the demulsibility of additive-modified lubricating oil compositions. It is a further object to add specific surfactants to the compounded lubricating oils to depress emulsification thereof in the presence of water. Other objects will be apparent from the following description in which parts and percentages, where used, are by weight.

According to the present invention, it has now been found that lubricating oil compositions containing detergent and/or other additives which promote emulsification of the oil with water may have such emulsifying tendencies reduced by adding to such compositions a surfactant organic compound having an acetylenic linkage, that is, an organic molecule having a triple bond carbon to carbon linkage ( $-\text{C}\equiv\text{C}-$ ). The compounds contemplated herein are hydroxy-substituted or halogen-substituted acetylenic hydrocarbons which are oil soluble within the effective ranges of amounts prescribed herein and which are normally solids or liquids at room temperature. These compounds generally contain from about 5 to about 18 carbon atoms, preferably from 6 to 10 carbon atoms and conform to the general formula:



where R represents a radical selected from the group consisting of hydrogen, a hydrocarbyl radical having from 3 to about 8 carbon atoms, a hydroxy-substituted hydrocarbyl radical containing from 3 to about 8 carbon atoms and a chloro-substituted hydrocarbyl radical containing from about 3 to about 8 carbon atoms, at least one R being a hydroxy- or chloro-substituted hydrocarbyl radical of from 3 to about 8 carbon atoms.

Specific examples of the acetylenic compounds contemplated herein are the following:

### 3-methyl 1-pentyne-3-ol



### 3-chloro-3-methyl-1-pentyne



2

### Ethynyl cyclohexanol



### 3,5-dimethyl 1-hexyn-3-ol



### 3-phenyl 1-butyl-3-ol



### 3-methyl 1-nonyn-3-ol



### 4-ethyl 1-octyn-3-ol



### 3,6-dimethyl-4-octyn-3,6-diol



The effectiveness of the invention has been demonstrated by adding typical acetylenic compounds to a lubricating oil composition and testing the resultant mixture for demulsibility, that is, the ability to obtain separation of water from oil-water mixtures. The test procedure used is the standard ASTM procedure designated as D1401-56T, in which 40 ml. of the oil composition being tested is mixed with 40 ml. of distilled water and the mixture is stirred for 5 minutes at 130° F. in a graduated cylinder, after which the resulting emulsion is allowed to stand at room temperature so that the emulsion breaks and forms separate layers of water, oil and emulsion. The time for the emulsion to be reduced to 3 ml. or less is noted as the measure of demulsibility.

### EXAMPLE 1

The first series of tests using this standard method were carried out with a fully formulated turbine circulating heavy oil composition containing about 100 parts of solvent-refined turbine oil base stock, 0.04 part of a rust inhibitor comprising a reaction product of tetrapropenyl succinic anhydride and oleic acid-triethylenetetramine reaction product, prepared after the fashion of Example 2, U.S. Patent No. 2,568,876, 0.25 part of di-t-butyl paracresol as an antioxidant and 0.15 part of zinc dihexyldithiophosphate as an antioxidant. The acetylenic compounds are added to the oil composition in the amounts shown, based on such composition, as set forth in Table 1, wherein the test results are shown.

TABLE I

|    |                                               | Time to 3 ml.<br>emul., min. |
|----|-----------------------------------------------|------------------------------|
| 65 | (A) Heavy turbine circulating oil composition | 59                           |
|    | (B) A+0.1% 3-methyl 1-pentyne-3-ol            | 51                           |
|    | (C) A+0.5% 3-methyl 1-pentyne-3-ol            | 52                           |
|    | (D) A+1.0% 3-methyl 1-pentyne-3-ol            | 50                           |
|    | (E) A+0.1% 3-chloro-3-methyl-1-pentyne        | 41                           |
| 70 | (F) A+0.5% 3-chloro-3-methyl-1-pentyne        | 34                           |
|    | (G) A+1.0% 3-chloro-3-methyl-1-pentyne        | 26                           |
|    | (H) A+0.1% ethynyl cyclohexanol               | 51                           |

|                                      | Time to 3 ml.<br>emul., min. |
|--------------------------------------|------------------------------|
| (I) A+0.5% ethynyl cyclohexanol      | 52                           |
| (J) A+1.0% ethynyl cyclohexanol      | 46                           |
| (K) A+0.1% 3,5-dimethyl 1-hexyn-3-ol | 50                           |
| (L) A+0.5% 3,5-dimethyl 1-hexyn-3-ol | 47                           |
| (M) A+1.0% 3,5-dimethyl 1-hexyn-3-ol | 43                           |
| (N) A+0.1% 3-phenyl 1-butyne-3-ol    | 51                           |
| (O) A+0.5% 3-phenyl 1-butyne-3-ol    | 49                           |
| (P) A+1.0% 3-phenyl 1-butyne-3-ol    | 38                           |

## EXAMPLE 2

A second series of tests were carried out as in Example 1, using a somewhat lighter oil blend containing about 100 parts of a lubricating oil base stock, 0.2 part zinc dihexyl-dithiophosphate as an antioxidant and 0.1 part of the same anti-rust agent used in Example 1, viz., the reaction product of tetrapropenyl succinic anhydride with the reaction product of triethylenetetramine and oleic acid. The results of these tests are shown in Table 2.

TABLE 2

|                                          | Time to 3 ml.<br>emul., min. |
|------------------------------------------|------------------------------|
| (A) Lubricating oil blend                | 42                           |
| (B) A+1.0% 3-methyl 1-pentyne-3-ol       | 36                           |
| (C) A+2.0% 3-methyl 1-pentyne-3-ol       | 36                           |
| (D) A+4.0% 3-methyl 1-pentyne-3-ol       | 35                           |
| (E) A+1.0% 3-methyl 1-nonyne-3-ol        | 25                           |
| (F) A+2.0% 3-methyl 1-nonyne-3-ol        | 17                           |
| (G) A+4.0% 3-methyl 1-nonyne-3-ol        | 16                           |
| (H) A+1.0% 3,5-dimethyl 1-hexyn-3-ol     | 28                           |
| (I) A+2.0% 3,5-dimethyl 1-hexyn-3-ol     | 27                           |
| (J) A+4.0% 3,5-dimethyl 1-hexyn-3-ol     | 24                           |
| (K) A+1.0% ethynyl cyclohexanol          | 24                           |
| (L) A+2.0% ethynyl cyclohexanol          | 25                           |
| (M) A+4.0% ethynyl cyclohexanol          | 22                           |
| (N) A+1.0% 3-phenyl 1-butyne-3-ol        | 27                           |
| (O) A+2.0% 3-phenyl 1-butyne-3-ol        | 26                           |
| (P) A+0.5% 4-ethyl 1-octyn-3-ol          | 32                           |
| (Q) A+1.0% 4-ethyl 1-octyn-3-ol          | 32                           |
| (R) A+1.5% 4-ethyl 1-octyn-3-ol          | 27                           |
| (S) A+2.0% 4-ethyl 1-octyn-3-ol          | 27                           |
| (T) A+0.2% 3,6-dimethyl-4-octyn-3,6-diol | 35                           |
| (U) A+0.3% 3,6-dimethyl-4-octyn-3,6-diol | 27                           |

It will be seen from Tables 1 and 2 that the acetylenic compounds of the invention are effective de-emulsifiers.

It will be understood that other acetylenic compounds

may be used in place of the acetylenic compounds shown in the tests with the same general demulsification results. The use of the acetylenic demulsifiers is highly advantageous since it permits the compounding of oils with many desirable additives that otherwise would render the oil blends emulsive. The invention is, therefore, not limited to the use of the acetylenic compounds with the specific additives shown in the tests. The amount of acetylenic compound may vary widely, ranging from about 0.1 to 10% of the weight of the oil blend or composition to which the compound is added. The range is preferably between about 0.1-5.0%. Higher amounts than about 10.0% are effective but may not be sufficiently economical to justify their use.

15. The present invention is applicable to the various lubricating oil compositions in which a base oil is blended with different detergents, corrosion inhibitors, antioxidants and the like. These oil compositions, chiefly because of these additives, tend to emulsify readily with water and the emulsions formed are difficult to break down so that oil can be separated from the water. The inclusion of relatively small amounts of one or more of the acetylenic compounds in the oil compositions tends to prevent emulsification altogether or to rapidly demulsify such emulsions as may be formed.

Having now fully described the invention, what is claimed as new and patentable is:

1. A lubricating oil composition comprising a major proportion of a lubricating oil and a minor proportion, from about 0.1% to about 10% by weight, of an acetylenic compound selected from the group consisting of 3-methyl-1-nonyne-3-ol, 3-phenyl-1-butyne-3-ol, and 3-chloro-3-methyl-1-pentyne.

2. The composition of claim 1, wherein the acetylenic compound is 3methyl-1-nonyne-3-ol.

3. The composition of claim 1, wherein the acetylenic compound is 3-phenyl-1-butyne-3-ol.

4. The composition of claim 1, wherein the acetylenic compound is 3-chloro-3-methyl-1-pentyne.

## References Cited by the Examiner

## UNITED STATES PATENTS

|           |        |          |           |
|-----------|--------|----------|-----------|
| 2,493,213 | 1/1950 | Altamura | 252-35    |
| 2,997,447 | 8/1961 | Russell  | 252-358 X |
| 3,095,381 | 6/1963 | Tinnon   | 252-331 X |

DANIEL E. WYMAN, Primary Examiner.

C. O. THOMAS, W. H. CANNON, Assistant Examiners.